

June 18, 1929.

J. K. SNYDER

1,717,946

PROCESS OF PRODUCING PRINTING SURFACES AND PRODUCTS THEREOF

Filed Nov. 29, 1927

*Fig. 1.*



INVENTOR  
Jacob K. Snyder  
BY  
Prindle, Wright, Neal & Bean  
ATTORNEYS

Patented June 18, 1929.

1,717,946

# UNITED STATES PATENT OFFICE.

JACOB K. SNYDER, OF GREENPOINT, NEW YORK, ASSIGNOR TO A. C. HORN COMPANY,  
A CORPORATION OF NEW YORK.

## PROCESS OF PRODUCING PRINTING SURFACES AND PRODUCTS THEREOF.

Application filed November 29, 1927. Serial No. 236,596.

My invention relates particularly to a process for reproducing by printing the grain of woods of various kinds, and the product thereof.

- 5 The object of my invention is to provide a process, and product thereof, for obtaining printing surfaces by the reproduction of the grain of various kinds of woods, whereby the grain of the wood may be applied to articles 10 of any desired kind, not only at a much smaller cost, but with a much more exact reproduction of the actual grain of the wood than has been possible in previous processes. The commercially used methods previously provided for this purpose involved the making 15 of a negative by the use of a plastic or molten material or electroplating or photography. Some of said processes required the etching of metal plates as the negatives and the making 20 of a positive from the negative. Furthermore, in the previous metal etching process it has been found that the depression and valleys caused by the etching are not sufficiently deep to hold enough ink for faithfully 25 reproducing the grain in exact detail when the ink is transferred to a roller and from the roller to the object to receive the grain. Also, the metal etching process is not adapted for application to curved surfaces, such as 30 moldings. In all the said previous processes there has been a loss of "value" and detail so as to prevent obtaining an exact replica of the original and said processes, furthermore, required very expensive equipment, materials and workmanship. The procedure in such previous processes always has 35 been to draw, engrave, photograph, or mold a fac-simile on a surface, to be transferred to stone, gelatine, metal or some other medium from which copies are to be printed or otherwise reproduced.

This invention comprises a method of using the grained wood itself as the negative so as to exactly reproduce the contours of wood 45 surfaces in each reproduction, thus copying the same with a fidelity and accuracy never attained before. The equipment used in my process is inexpensive, highly skilled labor is not required, depressions or valleys 50 are secured of sufficient depth for the roller to pick up from the surface sufficient ink to obtain therefrom an exact reproduction of the grain, and the process may be readily applied to curved surfaces. In connection 55 with my process it is found that not only is

sufficient ink picked up from the surface, but, due to the somewhat yielding character of the latter, enough ink is taken up by the roller to actually produce a raised printing surface when desired in the final printed 60 product.

In general, my invention involves the production of a negative of the grain on a wooden plate or molding of wood, which may be followed by deepening the valleys and depressions in the grain thereof so that the minutest detail of the same will be faithfully reproduced. 65

My invention is capable of being carried out in many different ways, but by way of 70 illustration I shall describe only certain ways of carrying out the same hereinafter.

By way of illustration I have shown certain portions of my invention in the accompanying drawings, in which— 75

Fig. 1 is a plan view of a veneered panel showing the same before being subjected to my process;

Fig. 2 is a cross-section of the same before treatment; 80

Fig. 3 is a cross-section of the same shown after the etching and in process of having a portion of the grain brushed out;

Fig. 4 is a plan view of the resultant panel after the treatment of brushing out and filling with ink has been completed; 85

Fig. 5 is a cross-section of the same after having had the ink introduced; and

Fig. 6 is a plan view of the inked panel showing a portion of the ink removed therefrom by a transfer roller. 90

My process may be applied to the reproduction of the grain of any desired kind of wood, but it has application especially to hard woods, such, for example, as mahogany, 95 walnut, oak, etc. Preferably a veneer 1 is made of one of these woods of sufficient thickness, as, for instance one inch, on a backing of any other desired kind of wood, such, for instance, as cross sectioned pine 2, in order 100 to obtain a wooden panel or molding in this manner that will not warp or distort in the course of the treatment. The veneer may be made from quarter-sawed sections or any other desirable cuts from the log and then 105 seasoned. The panel or molding is placed in a suitable form and is provided with a smooth level surface by abrasion or smoothing down with any desired tools. The surface is then treated with a material which will partially 110

- remove or soften or change parts of the wood grain so as to enable the latter to be brushed out with a wire or other stiff brush 3, having bristles of any desired material and of any desired length and degree of hardness, thus leaving depressions or valleys 4 of good depth and detail and the remainder or grain part of the surface in relief. By the degree of softening or etching and the degree of brushing, furthermore, the amount of depth to which the grain part of the fibre is to be removed may be readily controlled by the operator. For example, the material applied for softening the wood fibre may be, in the case of oak, a solution of 15 parts by weight of caustic soda in 100 parts by weight of water, which may be applied to the panel or molding for 8 hours. In the case of mahogany, a 99% strength by weight of acetic acid in water may be applied for 4 hours.
- After the softened parts of the wood have been brushed out in the manner above described, any excess of the softening material applied may be removed or neutralized so that any further etching action ceases. For example, where caustic soda has been used a 20% strength by weight of hydrochloric acid in water may be applied for a few minutes to neutralize the same, followed by washing in any desired way to remove the resulting materials. In the case where acetic acid has been used as the etching liquid, a 3% strength by weight of caustic soda in water may be applied thereto for a few minutes, followed by washing with water. Also, if desired, it will be understood that the etching materials may be removed either by brushing with water or an organic liquid such as naphtha or turpentine, if desired.
- After the valleys or depressions have been produced in the wood, in the above manner, it may be found that the negative thus obtained is somewhat soft for continued hard usage to withstand the wear of the ink scraper, and in that event a hardening treatment may be applied so as to harden the wood and thus enable innumerable impressions to be obtained without the ink being absorbed by the wood. For this purpose, for example, I may apply to the negative a 10% strength solution by weight of silver nitrate in water, or a 10% strength by weight of bichromate of potash in water, which, after having been applied to the negative may be precipitated or flocculated by the addition of an acid, base or salt solution, or by heat. In the case where silver nitrate is used, this may be done, for example, by applying a 10% strength by weight solution in water.
- If desired, furthermore, either with or without the previous hardening treatment, I may apply a treatment to the negative for water-proofing the same so as to prevent warping and distortion, as, for example, by providing therein a metallic salt of a fatty

acid, such as aluminum stearate, with a suitable binder, such as a resin or vegetable oil or cellulose ester carried in a solvent such as benzol, zylol, naphtha, turpentine, petroleum, etc. Such a water-proofing composition might be, for example, comprised of 6 parts by weight of aluminum stearate, 2 parts by weight of colophony resin, and 100 parts by weight of benzol.

The graining plate is then mounted on a specially constructed bed, a pliable bed, such as a mixture of glue, glycerine and formaldehyde, which acts in the double capacity of a cushion between the plate and the bed of sufficient resilience necessary for good reproduction and for the purpose of preventing the infiltration of moisture between the plate and the bed so as to prevent warping and twisting.

Thereafter, the negative obtained as above may have ink 5 of any desired color applied to the surface of the same with the aid of an ink scraper, so as to fill the depressions present therein, and a transfer roller 6 may be run over the surface so as to pick up the ink from the negative. Owing to the somewhat yielding character of the wood as compared with the metal negative, it will be found that the roller will pick up the design of the grain from the wood with the greatest faithfulness and detail. Thereupon the roller carrying the design of the grain in the ink, which has been received from the negative, may be applied to any surface provided for receiving the grain, as, for example, metal, paper, parchment, wood, cement, plaster, etc.

In the above process it will be understood, of course, that many other materials may be used instead of the materials mentioned above, and that the proportions of materials hereinabove mentioned may be varied widely, as desired, to suit the conditions applicable in the particular instance. For instance, instead of the caustic soda any other one of the known alkalies may be used, as, for example, caustic potash, lime, ammonia, etc. Also, instead of the acetic acid any other acid may be used, as, for example, hydrochloric, nitric, etc. For the neutralizing chemicals used any one of the alkalies may be used for neutralizing the etching acid and any one of the acids may be used for neutralizing the etching alkali. Furthermore, in place of the hardening materials, any other metal salt may be used. Likewise, instead of the aluminum stearate mentioned above any other fatty acid salt of a metal may be used. Many other resins may be used instead of the colophony resin above mentioned, and as the vegetable oil I may use, for example, linseed oil, china wood oil, etc. The cellulose ester mentioned may be cellulose nitrate or acetate, etc. Finally, instead of the solvents mentioned I may use any other suitable solvent applicable to the purpose.

While I have described my invention above

in detail I wish it to be understood that many changes may be made therein without departing from the spirit of the same.

I claim:

- 5 1. The process which comprises producing a printing surface by removing a part of the fibre from a wooden surface to place the grain in relief, by applying an etching material and then hardening the wooden surface and the printing from said surface.
- 10 2. The process which comprises producing a printing surface by removing a part of the fibre from a wooden surface to place the grain in relief, by applying an etching material and subjecting it to a water-proofing treatment and the printing from said surface.
- 15 3. The process which comprises producing a printing surface by removing a part of the fibre from a wooden surface of oak to place the grain in relief, by applying caustic soda

as an etching material, then brushing out the softened grain followed by neutralization of the etching material, then hardening the wooden surface by the application of a metallic salt, then adding a precipitant and subjecting the surface to a water-proofing treatment with a metallic stearate and a binder in liquid phase and the printing from said surface.

25 4. A printing surface of wood carrying depressions to place the grain of the wood, in relief, and a water-proofed grain.

5. A printing surface of wood carrying depressions to place the grain of the wood in relief, and a hardened grain impregnated with a metal salt and water-proofed by the presence of a metallic stearate and a binder.

In testimony that I claim the foregoing, I have hereunto set my hand this 17th day of November, 1927.

JACOB K. SNYDER.